

## UNITED STATES PATENT OFFICE

AUGUSTE HOLLARD, OF PARIS, FRANCE, ASSIGNOR TO SOCIÉTÉ NOUVELLE DE L'ORFÈVRERIE D'ERCUIS, OF PARIS, FRANCE, A CORPORATION OF FRANCE

## CHROMIUM PLATING BY ELECTROLYTIC DEPOSITION

No Drawing. Application filed December 21, 1928, Serial No. 327,749, and in France January 12, 1928.

The present invention relates to chromatizing by electrolytic deposition; and it consists in arranging the body to be coated at the cathode of an electrolytic bath composed of 5 an aqueous solution of sodium bichromate, chromic acid and chromium fluoborate.

The proportions of the substances which enter into the composition of the bath should not differ substantially from the following, 10 which are given, by way of example, for a 100-liter bath:

|                          |          |
|--------------------------|----------|
| Sodium bichromate.....   | 25 kgs.  |
| Chromic acid.....        | 15 kgs.  |
| Chromium fluoborate..... | 900 grs. |

15 This bath operates with chromium anodes—that is to say, with anodes which are soluble in the bath—or with insoluble anodes, lead for example.

20 The preferred density of the current varies from 10 to 20 amperes per square decimeter of cathode, and the preferred temperature of the bath ranges about 45° C.

I claim as my invention:—

25 A bath for chromium plating conductive bodies by electrolytic deposition comprising sodium bichromate, 25 kilograms; chromic acid, 15 kilograms; and chromium fluoborate, 900 grams.

30 AUGUSTE HOLLARD.